

[72] Inventor **Gerhard Wolfrum**  
**Opladen, Germany**

[21] Appl. No. **867,916**

[22] Filed **Oct. 20, 1969**

[45] Patented **Dec. 28, 1971**

[73] Assignee **Farbenfabriken Bayer Aktiengesellschaft**  
**Leverkusen, Germany**

[32] Priority **Oct. 19, 1968**

[33] **Germany**

[31] **P 18 04 133.3**

3,110,696 11/1963 **Dexter.....** 260/45.8  
 3,399,027 8/1968 **Siegrist et al. ....** 8/31  
 3,547,646 12/1970 **Hori et al. ....** 96/90

**Primary Examiner—George F. Lesmes**  
**Assistant Examiner—Patricia C. Ives**  
**Attorney—Plumley, Tyner & Sandt**

**ABSTRACT:** Dyeing and printing of textile materials of metal-containing polypropylene with compounds of the general formula



in which A stands for a optionally substituted benzene or naphthalene radical the -OH-group and the substituent -CH-N- being attached to adjacent carbon atoms; B represents a optionally substituted benzene or naphthalene the substituent -OR and the substituent



being attached to adjacent carbon atoms and R representing an alkyl radical A and B cannot simultaneously represent radicals of the benzene series.

**[54] PROCESS FOR THE DYEING AND PRINTING OF METAL-CONTAINING POLYOLEFIN TEXTILE MATERIALS**

**2 Claims, No Drawings**

[52] U.S. Cl. .... **8/31, 8/180,**  
**260/558**

[51] Int. Cl. .... **D06p 1/36,**  
**C09b 65/00**

[50] Field of Search. .... **8/41, 31,**  
**180-181; 260/558**

**[56] References Cited**

UNITED STATES PATENTS

2,767,173 10/1956 **Katz** ..... **260/240**

**PROCESS FOR THE DYEING AND PRINTING OF METAL-  
CONTAINING POLYOLEFIN TEXTILE MATERIALS**

It has been found that materials of metal-containing polyolefins, such as filaments, fibers, foils, woven and knitted fabrics, especially those of nickel-containing polypropylene, can be dyed and printed fast when they are treated with compounds of the general formula



under conditions known in dyeing and printing industry.

In the general formula, A stands for a benzene or naphthalene radical which may be further substituted by chlorine or bromine, or by alkyl radicals with one to four carbon atoms, the —OH— group and the substituent —CH—N—... being attached to adjacent carbon atoms. B stands for a benzene or naphthalene nucleus which may be substituted by chlorine or bromine, or by alkyl radicals with one to four carbon atoms or alkoxy groups with one to four carbon atoms, the substituent —OR and the substituent



being attached to adjacent carbon atoms, R represents an alkyl radical with one to four carbon atoms; A and B cannot simultaneously represent radicals of the benzene series.

The individual process according to the invention is carried out in such a manner that the compounds of the general formula (I) are applied on to the materials to be treated, particularly fibers and fabrics, from acidic, neutral or weakly alkaline suspensions, dispersions, pastes or solutions, preferably with the use of dispersing agents, emulsifiers, dyeing accelerators, thickening agents and/or levelling auxiliaries, from a dyebath, a padding liquor or by means of a printing paste. When a dyeing liquor is used, this is brought to an elevated temperature for a certain time by gradually raising the temperature in the course of the dyeing process, for example, to temperatures of about 90°–140° C., preferably to temperatures of about 95°–110° C. When a padding liquor is used, the padded fabric is subsequently subjected to a heat treatment, if necessary, after an intermediate drying. When a printing paste is used, the fabric is likewise subjected to a heat treatment after printing. The heat treatment may be carried out either by hot air or by steam, at temperatures of, for example, 100°–140° C. The duration of the treatment is generally about 1–10 minutes. The resistance to rubbing of the dyeings obtained can sometimes be improved by an alkaline after-treatment of the dyed material, or by an after-treatment with reducing agents, such as sulfites or formaldehyde/sulphite addition products in an alkaline medium, optionally with the addition of an emulsifier.

Suitable dispersing or emulsifying agents which are advantageously added to the compounds of the formula (I) to be used according to the invention are commercially available products, such as sulfite cellulose waste liquor products, condensation products of higher alcohols and ethylene oxide, soaps, polyglycol ethers of fatty acid amides, formaldehyde condensation products of aromatic sulfonic acids or mixtures of such compounds.

To produce printing pastes which contain the compounds of the formula (I) to be used according to the invention, the customary thickening agents, such as methyl cellulose, carob bean flour, crystal gum, alginates or tragacanth can be used. The printing pastes may also contain the usual additives, such as urea, thiourea, thiodiglycol, methylated alcohols, sodium-m-nitrobenzosulphonate or aqueous emulsions of sulfonated oils.

The dyed or printed materials, preferably obtained from metal-containing polypropylene, can be after-treated in usual manner, subsequently to the dyeing or printing process, for example, by washing, brightening, decatizing or heat setting.

The process according to the invention is preferably used for the dyeing and printing of metal-containing, preferably nickel-containing, polypropylene fiber materials. The term metal-containing polypropylene fiber materials comprises those fiber materials which contain the metals either as such or in the form of their salts, but preferably in the form of chelates. Suitable metal chelates are particularly nickel chelates or nickel compounds of phenols, bis-(alkyphenol)-monosulfides, bis-(p-alkyphenol)-sulfoxides, bis-(p-alkyphenol)-

10 sulphones dithiocarbamates, o-hydroxyphenyl-benztriazoles, hydroxamic acids, and nickel dimethyl dioxime and nickel acetylacetone, at concentrations of 0.01 to 3 percent, preferably 0.1 to 2 percent. The nickel complexes can be used by themselves or in admixture with other nickel complexes or nickel salts. Instead of the nickel compounds mentioned above, the polypropylene materials may also contain salts or chelates of zinc, aluminum, magnesium, cobalt, copper or chromium by themselves or in admixture with one another. Finally, the last-mentioned metal salts or chelates may also be present together in the polypropylene fiber materials in admixture with the above-mentioned salts or chelates of nickel.

15 The compounds of the general formula (I) to be used according to the invention are obtained in known manner by reacting o-hydroxyaldehydes of the benzene or naphthalene series with o-alkoxy-carboxylic acid hydrazides of the benzene or naphthalene series.

20 The following o-hydroxyaldehydes may be used; for example: 2-hydroxy-benzaldehyde, 3-methoxy-2-hydroxy-benzaldehyde, 5-chloro-2-hydroxybenzaldehyde, 3,5-dichloro-2-hydroxybenzaldehyde, 5-bromo-2-hydroxybenzaldehyde, 2-hydroxy-naphthaldehyde-(1), 1-hydroxy-naphthaldehyde-(2), 2-hydroxy-naphthaldehyde-(3), 5-chloro-2-hydroxy-naphthaldehyde-(1), 6-chloro-2-hydroxy-naphthaldehyde-(1), (7-chloro-2-hydroxy-naphthaldehyde-(1), 6-bromo-2-hydroxy-naphthaldehyde-(1), 6-methyl-2-hydroxy-naphthaldehyde-(1), 2-methoxy-2-hydroxy-naphthaldehyde-(1).

25 The following o-alkoxy-carboxylic acid hydrazides may be used, for example: 2-methoxybenzoic acid hydrazide, 2-ethoxybenzoic acid hydrazide, 2-propoxybenzoic acid hydrazide, 2-

30 n-butoxybenzoic acid hydrazide, 2-methoxy-5-methylbenzoic acid hydrazide, 2-methoxy-4-methylbenzoic acid hydrazide, 2-methoxy-4-n-butyl-benzoic acid hydrazide, 2-methoxy-5-chloro-benzoic acid hydrazide, 2-methoxy-4-chloro-benzoic acid hydrazide, 2-methoxy-3-methyl-5-chloro-benzoic acid hydrazide, 2-methoxy-4,6-dimethylbenzoic acid hydrazide, 2-

35 ethoxy-5-methylbenzoic acid hydrazide, 2-ethoxy-4-methylbenzoic acid hydrazide, 2-ethoxy-5-tert.butyl-benzoic acid hydrazide, 2-ethoxy-5-chloro-benzoic acid hydrazide, 2-ethoxy-3-methyl-5-chloro-benzoic acid hydrazide, 2-ethoxy-5-methyl-4-chloro-benzoic acid hydrazide, 2,3-diethoxybenzoic acid hydrazide, 2-n-butoxy-5-chloro-benzoic acid hydrazide, 1-methoxy-naphthalene-carboxylic acid-(2)-hydrazide, 2-methoxy-naphthalene-carboxylic acid-(1)-hydrazide,

40 2-methoxy-naphthalene-carboxylic acid-(3)-hydrazide, 1-ethoxy-naphthalene-carboxylic acid-(2)-hydrazide, 2-ethoxy-naphthalene-carboxylic acid-(1)-hydrazide, 2-ethoxy-naphthalene-carboxylic acid-(3)-hydrazide.

45 Compounds suitable for the process according to the invention are, for example, the compounds set out in the following table.

| Compound No. | TABLE                                                                                |                                                                                       |
|--------------|--------------------------------------------------------------------------------------|---------------------------------------------------------------------------------------|
|              | Compounds of the formula—                                                            |                                                                                       |
|              | $D-CH=N-N-C-E$<br> <br>H O                                                           |                                                                                       |
| 1            |  |  |

| Compound No. | D                                                                                   | E                                                                                   |
|--------------|-------------------------------------------------------------------------------------|-------------------------------------------------------------------------------------|
| 2            | Same as above                                                                       |    |
| 3            | do                                                                                  |    |
| 4            |    |    |
| 5            | do                                                                                  |                                                                                     |
| 6            | do                                                                                  |                                                                                     |
| 7            | do                                                                                  |                                                                                     |
| 8            |   |    |
| 9            | Same as above                                                                       |  |
| 10           | do                                                                                  |  |
| 11           | do                                                                                  |  |
| 12           | do                                                                                  |  |
| 13           | do                                                                                  |  |
| 14           | do                                                                                  |  |
| 15           |  |  |
| 16           | Same as above                                                                       |  |

| Compound No. | D                                                                                     | E                                                                                     |
|--------------|---------------------------------------------------------------------------------------|---------------------------------------------------------------------------------------|
| 17           | do                                                                                    |    |
| 18           | do                                                                                    |    |
| 19           |    |    |
| 20           | do                                                                                    |    |
| 21           | do                                                                                    |    |
| 25           |                                                                                       |                                                                                       |
| 22           | Same as above                                                                         |    |
| 30           |                                                                                       |                                                                                       |
| 35           |   |   |
| 40           |  |  |
| 45           | do                                                                                    |                                                                                       |
| 50           | do                                                                                    |  |
| 55           | do                                                                                    |  |
| 60           | Same as above                                                                         |  |
| 65           | do                                                                                    |  |
| 70           |                                                                                       |                                                                                       |

Preferred compounds of the general formula (I) are those in which A stands for a naphthalene radical substituted as indicated, and B stands for a benzene ring substituted as indicated; as well A as B may contain the further substituents mentioned above.

The dyeings obtained by the process according to the invention are distinguished by outstanding fastness to washing, solvents and heat setting as well as by very good fastness to light.

The subject matter of the invention further comprises compounds of the formula



in which X stands for a 2-methoxyphenyl, 2-methoxy-4-methylphenyl, 2-methoxy-5-methylphenyl, 2-methoxy-2-tert.-butylphenyl, 2-methoxy-5-chlorophenyl or 2-methoxy-naphthyl radical.

The parts or percentages given in the following examples are parts by weight or percentages by weight.

#### EXAMPLE 1

Ten parts of a commercial, nickel-containing polypropylene yarn are dyed at boiling temperature for 1 hour in a bath which contains, in 400 parts water, 0.1 part of the finely dispersed compound of the formula



as well as 0.2 parts of a naphthalene-sulfonic acid/formaldehyde condensation product and 0.3 parts of a 30 percent aqueous acetic acid. The dyed yarn is then rinsed first with hot then with cold water and finally after-treated at 50°C. with the addition of 0.5 parts/liter of a commercial detergent. After rinsing and drying, a clear greenish yellow dyeing of very good fastness to washing, rubbing, solvents and light is obtained.

#### EXAMPLE 2

A fabric of nickel-containing polypropylene is printed with a printing paste of the following composition:

20 parts of a finely dispersed compound of the formula



260 parts of water,  
500 parts of a thickening agent based on tragacanth,  
100 parts of urea,  
120 parts of a 50 percent aqueous ammonium sulfate solution,  
1,000 parts.

The printed fabric is dried and subsequently steamed at 100°C. for 30 minutes. After thoroughly rinsing and an after-treatment at 50°-80°C. with 0.5 parts, per liter water, of a reaction product of about 8-10 mol ethylene oxide with 1 mol nonylphenol, rinsing and drying, a clear greenish yellow print with very good fastness properties is obtained.

When the compound described in example 1 is replaced by one of the compounds of the formula (I) obtainable by the reaction of the compounds (II) and the compounds (III) set out in the table below for the dyeing or printing according to example 1 or 2, there are obtained, on nickel-containing polypropylene, dyeings of shades specified in the last column, which also have very good fastness properties.

TABLE

|    | II                                                                       | III                                                                                                         |                                          |
|----|--------------------------------------------------------------------------|-------------------------------------------------------------------------------------------------------------|------------------------------------------|
| 5  | (o-Hydroxylaldehyde)                                                     | (o-Alkoxycarboxylic acid hydrazide)                                                                         | Shade on nickel-containing polypropylene |
| 10 | 1-hydroxy-2-naphth-aldehyde<br>Do                                        | 2-methoxy-benzoic acid hydrazide,<br>2-methoxy-5-methyl-benzoic acid hydrazide                              | Yellow.<br>Do.                           |
| 15 | 2-hydroxy-1-naphth-aldehyde<br>Do                                        | 2-ethoxy-benzoic acid hydrazide,<br>2-n-butoxy-benzoic acid hydrazide                                       | Greenish yellow.<br>Do.                  |
| 20 | Do                                                                       | 2-methoxy-4-methylbenzoic acid hydrazide,<br>2-methoxy-5-methylbenzoic acid hydrazide                       | Do.                                      |
| 25 | Do                                                                       | 2-methoxy-6-tert.-butylbenzoic acid hydrazide,<br>2-methoxy-5-chlorobenzoic acid chloride                   | Do.                                      |
| 30 | Do                                                                       | 2-methoxy-3-methyl-5-chloro-benzoic acid hydrazide,<br>2,3-dimethoxybenzoic acid hydrazide                  | Do.                                      |
|    | 1-hydroxy-2-naphth-aldehyde<br>Salicylaldehyde                           | 2-methoxynaphthalene-3-carboxylic acid hydrazide,<br>2-methoxynaphthalene-3-carboxylic acid hydrazide<br>do | Slightly greenish yellow.<br>Do.         |
|    | Do                                                                       | 1-methoxynaphthalene-2-carboxylic acid hydrazide,<br>2-methoxynaphthalene-3-carboxylic acid hydrazide<br>do | Strongly greenish yellow.<br>Do.         |
|    | 2-hydroxy-3,5-dichloro-benzaldehyde,<br>3-methoxy-2-hydroxy-benzaldehyde | 2-methoxynaphthalene-3-carboxylic acid hydrazide<br>do                                                      | Greenish yellow.<br>Do.                  |

#### I claim:

1. Process for the dyeing and printing of textile materials of metal-containing polypropylene, which comprises applying to the textile materials a compound of the general formula



in which A stands for a benzene or naphthalene radical which is unsubstituted or which is substituted by chlorine or bromine, or by alkyl radicals with one to four carbon atoms, the—OH—group and the substituent—CH—N— being attached to adjacent carbon atoms; B represents a benzene or naphthalene radical which is unsubstituted or which is substituted by chlorine or bromine, or by alkyl radicals with one to four carbon atoms, or by alkoxy groups with one to four carbon atoms, the substituent—OR and the substituent



being attached to adjacent carbon atoms and R representing an alkyl radical with one to four carbon atoms; A and B cannot simultaneously represent radicals of the benzene series.

2. Process of claim 1 wherein said compound is of the formula



in which X stands for a 2-methoxyphenyl, 2-methoxy-4-methylphenyl, 2-methoxy-5-methylphenyl, 2-methoxy-5-tert.-butylphenyl, 2-methoxy-5-chlorophenyl or 2-methoxy-naphthyl radical.

\* \* \* \* \*

UNITED STATES PATENT OFFICE  
CERTIFICATE OF CORRECTION

Patent No. 3,630,656 Dated December 28, 1971  
SN 867,916  
Inventor(s) Gerhard Wolfrum

It is certified that error appears in the above-identified patent and that said Letters Patent are hereby corrected as shown below:

Page 1, Abstract, at second line following general formula:

change -CH- to -CH=

| <u>Column</u> | <u>Line</u> |                                                                                                                                                                                          |
|---------------|-------------|------------------------------------------------------------------------------------------------------------------------------------------------------------------------------------------|
| 1             | 20          | change CH N to CH=N                                                                                                                                                                      |
| 2             | 10          | change "sulfones dithiocarbamates"<br>to sulfones, dithiocarbamates                                                                                                                      |
| 2             | 50          | change "2-ethoxy4-methyl"<br>to 2-ethoxy-4-methyl                                                                                                                                        |
| 2             | 77          | change "  "<br>to  |
| 2             | 34          | change "(1), (7 -" to (1), 7 -                                                                                                                                                           |

UNITED STATES PATENT OFFICE  
CERTIFICATE OF CORRECTION

-2-

Patent No. 3,630,656 Dated December 28, 1971

Inventor(s) Gerhard Wolfrum

It is certified that error appears in the above-identified patent and that said Letters Patent are hereby corrected as shown below:

| <u>Column</u> | <u>Line</u>        |                                                                                              |
|---------------|--------------------|----------------------------------------------------------------------------------------------|
| 3             | Compound<br>7 (E)  | change "   |
|               |                    | to         |
| 3             | Compound<br>13 (E) | change "  |
|               |                    | to       |

UNITED STATES PATENT OFFICE  
CERTIFICATE OF CORRECTION

Patent No. 3,630,656 Dated December 28, 1971

Inventor(s) Gerhard Wolfrum

It is certified that error appears in the above-identified patent and that said Letters Patent are hereby corrected as shown below:

| <u>Column</u> | <u>Line</u> |                                                                                                |
|---------------|-------------|------------------------------------------------------------------------------------------------|
| 3             | 70          | change "  OH |
|               |             | to          |
| 5             | 15          | change "2-methoxy-2-"<br>to 2-methoxy-5-                                                       |

UNITED STATES PATENT OFFICE  
CERTIFICATE OF CORRECTION

-4-

Patent No. 3,630,656 Dated December 28, 1971

Inventor(s) Gerhard Wolfrum

It is certified that error appears in the above-identified patent and that said Letters Patent are hereby corrected as shown below:

| <u>Column</u> | <u>Line</u> |                                                        |                                                                                                                         |
|---------------|-------------|--------------------------------------------------------|-------------------------------------------------------------------------------------------------------------------------|
| 5             | 17          | change                                                 | "naphtyl"                                                                                                               |
|               |             | to                                                     | naphthyl                                                                                                                |
| 6             | Claim 1     | first formula, change                                  |                                                                                                                         |
|               |             |                                                        | "A CH N N C B"                                                                                                          |
|               |             | to                                                     | A-CH=N-N-C-B                                                                                                            |
| 6             | 45          | change                                                 | "-CH N-"                                                                                                                |
|               |             | to                                                     | -CH=N-                                                                                                                  |
| 6             | 52          | change                                                 | "C NH<br>"<br>O                                                                                                         |
|               |             | to                                                     | -C-NH-<br>"<br>O                                                                                                        |
| 6             | 65          | change<br>formula to<br>(not<br>clearly<br>reproduced) | "<br><br>CH=N-N-CO-X<br>"<br>H<br>" |

UNITED STATES PATENT OFFICE  
CERTIFICATE OF CORRECTION

Patent No. 3,630,656 Dated December 28, 1971

Inventor(s) Gerhard Wolfrum

It is certified that error appears in the above-identified patent and that said Letters Patent are hereby corrected as shown below:

The following errors were made by applicants. Our check in the amount of \$15.00 is enclosed.

Column      Line

1      26      change " - O - NH - "  
                    |  
                    O  
                    |  
                    to      - C - NH -  
                    |  
                    O

5      10      change "       - CH = N - N - CO - X      "  
                    |  
                    OH  
                    to       - CH = N - N - CO - X  
                    |  
                    OH      H

Signed and sealed this 12th day of September 1972.

(SEAL)  
Attest:

EDWARD M.FLETCHER, JR.  
Attesting Officer

ROBERT GOTTSCHALK  
Commissioner of Patents